# EUROPEAN PATENT SPECIFICATION

(11) **EP 0 898 513 B1**
(45) Date of publication and mention of the grant of the patent: **16.08.2000**
(21) Application number: 97923210.5
(22) Date of filing: 19.05.1997
(51) Int. Cl.: B41M 3/00, D21H 21/28, B41M 1/10, B41M 1/12

(54) **PAPER TREATMENT**
VERFAHREN ZUR BEHANDLUNG VON PAPIER
TRAITEMENT DU PAPIER

(30) Priority: 18.05.1996 GB 9610456
(43) Date of publication of application: 03.03.1999
(73) Proprietor: Watson Grange Limited, London EC4Y 0HP (GB)
(72) Inventor: FORBES, Stephen, Glenrothes TY6 3QF (GB)
(74) Representative: Wise, Stephen James
(86) International application number: GB9701378
(87) International publication number: WO9744195

(56) References cited:
- EP-A- 0 414 015
- EP-A- 0 601 517
- DE-A- 4 307 873
- DE-C- 67 632
- FR-A- 537 357
- US-A- 2 089 949

## Description

This invention relates to colouring papers and cards particularly, but not exclusively, for use in book binding and the manufacture of games boards, presentation boxes and stationery.

The cost of coloured dyes accounts for a significant proportion of the cost of producing coloured paper. This is particularly so for deep coloured papers which require high dye concentration.

Attempts have been made in the past to print a layer of deeply coloured ink on to the entire surface of a sheet of lightly coloured paper to achieve a deep colour surface. The layer of ink printed on to the surface is made as thin as possible to minimise the amount of ink required. However, printing papers of this kind tend to scuff easily and are unsuitable for many purposes; the surface ink is easily damaged or scraped off, for example when the paper is scuffed or folded. This reveals an unsightly line and renders the colour of the base paper visible.

It is also known to form a paper product of a dyed, deeply coloured surface ply and a lightly coloured backing ply. A disadvantage of such papers is the cost of producing same, given the multiply structure.

EP 0,414,015 discloses a method of colouring paper in which the upper surface of a tissue web is impregnated with a colouring ink in a single application. The degree of penetration of the ink is limited as much as possible, and there is no teaching concerning the rate of decrease in concentration of the ink through the depth of the tissue web.

An object of the present invention is to provide a deeply coloured paper that is durable, while still being cost effective to produce. This is achieved by impregnating the paper with ink or dye below the upper or outer surface of the paper, and using a technique to do this which optimises the concentration of the impregnated ink relative to the depth of penetration below the upper layer of the paper.

According to a first aspect, the present invention provides a paper product comprising a ply of lightly coloured base paper having an upper surface in which a portion of the ply below the upper surface is impregnated with a colouring ink, wherein the colouring ink decreases in concentration in a direction through the ply moving away from the upper surface, characterised in that the rate of the decrease in concentration of the ink is greater in a first portion of the paper product closest to the upper surface than in a second portion of the paper product further away from the upper surface.

Preferably the concentration of impregnated ink decreases at a first substantially linear rate through the first portion of the paper produce closest to the upper surface of the product, and at a second and lower substantially linear rate through the second portion of the paper product further away from the upper surface.

The paper product may be a cellulosic fibre paper, a paper made of a synthetic fibre material or a paper made of mixed fibres.

The colouring ink may extend substantially across the entire surface area of the paper product.

The product may be capable or adapted to be folded so as to form a crease in the product such that the resulting damage to the outermost fibres towards the upper surface does not allow uncoloured fibres to show through.

The lightly coloured paper base may be white or tinted.

The paper product may have more than one ply of paper. The colouring ink may be present only in the top ply; it may extend substantially or wholly through the top ply.

The presence of the colouring ink below the surface of the ply may allow the product to be folded without the base colour of the product showing through the surface of the top ply. The type of coloured ink is preferably chosen so as to have a good scuff resistance.

The ink is preferably selected to have one or more of the following characteristics:
a. high resistance to dry and moist rub;
b. high resistance to colour change under pressure and temperature;
c. flexibility of ink film for embossing and casing-in so as to prevent cracking of the ink layer;
d. good foil stamping, blind blocking and screen printing properties;
e. good lightfastness (ie resistance to fading, for example 3 min on the Blue Wool Scale);
f. no set-off onto underside;
g. no set-off onto design rolls or matrix bowls;
h. good paper penetration characteristics.

The ink may be solvent based but is preferably water based.

The ink may penetrate to a depth of at least 30 or 35 microns below the upper surface of the paper product. It may penetrate to a greater depth. The ink may penetrate to a depth of substantially 30% of the depth of the ply below the upper surface of the paper product. It may have a penetration of at least 30% and may have a greater penetration. If the ink is solvent based then the penetration may be greater. The concentration of ink may decrease with depth of penetration.

Traditional printing methods inevitably result in some ink penetrating into the paper. Nevertheless, printers generally seek to minimise the quantity of ink that is used. This is done by formulating the ink to minimise ink penetration into the paper and/or by coating, treating or selecting the paper so as to minimise ink penetration.

A paper product in accordance with the present invention preferably has a greater ink penetration; in one of its aspects, the invention seeks to achieve a certain or minimum ink penetration to obtain the advantages discussed.

According to a second aspect, the present invention provides a method of producing a paper product including the steps of:
a) printing with ink a sheet surface of the paper product;
b) allowing the ink to permeate into a portion of the paper product below the sheet surface; and
c) reprinting the sheet with ink, so that the rate of the decrease in concentration of the ink is greater in a first portion of the paper product closest to the upper surface than in a second portion of the paper product further away from the upper surface.

The method may also include one or more of the following steps:
a. unwinding the paper product;
b. drying the ink between the two printing applications;
c. applying a lacquer over the sheet surface;
d. embossing the product;
e. re-moisturising the underside of the product;
f. rewinding the product;
g. allowing a dwell time to re-stabilise the product, for example prior to rewinding it.

The method may be performed on a paper making machine, for example, immediately after the drum reel operation. Alternatively, the method may be performed on a paper product removed from a paper making machine.

An embodiment of the invention will now be described, by way of example only, with reference to the accompanying drawings of which:
Fig 1 is a cross section through a paper product;
Fig 2 is a graph of ink concentration through the paper product ;
Fig 3 is a schematic cross section of an apparatus for producing the product; and
Fig 4 is a graph of ink concentration through a paper product produced by the apparatus of Figure 3.

The two ply paper product 10 of Fig 1 has been overprinted over its entire upper surface 20 with an ink 21. The ink penetrates from the top surface 20 substantially through the upper ply 11 but not into the lower ply 12. A thin layer of ink 21 is present at the top surface 20 and, as shown in Fig 2, the concentration of ink x decreases in a direction y moving away from the top surface.

The plies 11,12 may be of a light colour having been dyed during manufacture or may be white; they may be of different colours. The plies 11,12 may be of a corresponding lighter colour to the ink; for example, the plies may be light blue when the ink is a deep or dark blue.

The paper product 10 is sufficiently strong that it can be used as a binding paper for example for booking binding, games boards, box and stationery manufacturing. Its presentation surface has adequate scuff and water resistance so that it does not readily lose colour or deposit fibres when a contacting surface is rubbed against it. The paper accepts adhesives (for binding purposes) whilst not permitting the adhesive to saturate the sheet. Preferably, the scuff resistance is such that face to face abrasion resistance carried out on Martindale testing equipment is in excess of 1000 cycles. The ink is adequately absorbed into the paper such that when the paper is folded over an edge or corner, the resulting damage to the outermost layer of fibres does not allow uncoloured fibres to show through.

The ink may be an aqueous based ink.

The apparatus 30 of Fig 3 is arranged to treat a roll of paper 31 which has been manufactured in a separate process. The apparatus 30 comprises:
a. an unwinding station 32;
b. a first printing station 33 having a printing head for applying ink across the entire surface of the paper product;
c. an infra-red or microwave drying station 34;
d. a second printing station 35 having a printing head for applying ink across the entire surface of the paper product;
e. a second infra-red or microwave drying station 36;
f. an embossing nip 37;
g. a station 38 for applying a layer of lacquer across the paper product;
h. a backwet unit or re-moisturising station 39;
i. an accumulator 40; and
j. a rewind station 41.

The paper product passes through a dwell portion 39,40 to allow the sheet adequate dwell time such that it re-stabilises before being rewound.

The application of an aqueous based ink to one side of the paper tends to induce a "positive" curl ie the bias of the curve is towards the overprinted paper surface. If the paper was simply embossed and then rewound it would be likely to be unstable at the sheeting process. In order to alleviate the influence of the overprinted ink and thus the tendency to curl, the re-moisturising station 39 which may comprise a re-moisturising unit and a conditioning unit is stationed prior to rewinding. The re-moisturising unit applies water to the uncoated paper surface thereby counteracting the influence of the water-based overprint ink. The conditioning unit allows the paper sufficient dwell time in the process to accept the moisture and re-stabilise.

Whilst the ink may be applied to the paper product in a single printing operation it has been found advantageous to apply the ink in two separate passes with an intervening drying operation. The drying operation may be encouraged by use of an infra-red or microwave dryer (as illustrated) but such a dryer is not always necessary.

Typically, 3 grams per m² dry ink may be applied to the paper product. In the embodiment of Fig 3 this may be achieved by applying 1.5 grams per m² at each of the two print heads.

The use of two (or more) printing stages results in a different and indeed more preferable ink concentration distribution than that shown in Figure 2. Figure 4 graphs the concentration from a two print process.

In likeness to Figure 2, the line AB represents the concentration of the ink relative to the depth of the paper below the upper sheet surface after the first print run. However, the very presence of the impregnated ink from the first print run varies the rate of impregnation of the ink from the second print run, and this is depicted by line CD. The resultant aggregate concentration from the two print runs is therefore graphed by the line AD.

This concentration is advantageous as the ink concentration is greatest, exponentially, where it is most wanted. It reduces the amount of ink needed to achieve a paper of suitable durability and this is beneficial in light of the aforementioned high cost of the ink itself.

Additional passes of the paper through successive printing heads is also possible within the invention. Further modifications are also envisaged without departing from the scope of the claims.

## Claims

1. A paper product comprising a ply of lightly coloured base paper having an upper surface in which a portion of the ply below the upper surface is impregnated with a colouring ink, wherein the colouring ink decreases in concentration in a direction through the ply moving away from the upper surface, characterised in that the rate of the decrease in concentration of the ink is greater in a first portion of the paper product closest to the upper surface than in a second portion of the paper product further away from the upper surface.

2. A paper product as claimed in Claim 1 wherein the concentration of impregnated ink decreases at a first substantially linear rate through said first portion of the paper product closest to the upper surface of the product, and at a second and lower substantially linear rate through said second portion of the paper product further away from the upper surface.

3. A paper product as claimed in Claim 1 or Claim 2 made from cellulosic, synthetic or mixed fibres.

4. A paper product as claimed in any one of the preceding Claims wherein the colouring ink extends substantially across the entire surface area of the paper product.

5. A paper product as claimed in any one of the preceding claims capable or adapted to be folded so as to form a crease in the product such that the resulting damage to the outermost fibres towards the upper surface does not allow uncoloured fibres to show through.

6. A paper product as claimed in any one of the preceding Claims wherein the lightly coloured paper base is tinted.

7. A paper product as claimed in any one of the preceding Claims having more than one ply of paper and wherein the colouring ink is present only in the top ply.

8. A paper product as claimed in any one of the preceding Claims wherein the colouring ink is selected to have one or more of the following characteristics:
a. high resistance to dry and moist rub;
b. high resistance to colour change under pressure and temperature;
c. flexibility of ink film for embossing and casing-in so as to prevent cracking of the ink layer;
d. good foil stamping, blind blocking and screen printing properties;
e. good lightfastness (ie resistance to fading, for example 3 min on the Blue Wool Scale);
f. no set-off onto underside;
g. no set-off onto design rolls or matrix bowls;
h. good paper penetration characteristics.

9. A paper product as claimed in any one of the preceding Claims wherein the colouring ink penetrates to a depth of at least 30 microns below the upper surface of the paper product.

10. A method of producing a paper product including the steps of:
a) printing with ink a sheet surface of the paper product;
b) allowing the ink to permeate into a portion of the paper product below the sheet surface; and
c) reprinting the sheet with ink, so that the rate of the decrease in concentration of the ink is greater in a first portion of the paper product closest to the upper surface than in a second portion of the paper product further away from the upper surface.

11. A method as claimed in Claim 10 also including one or more of the following steps:
a. unwinding the paper product;
b. drying the ink between the two printing applications;
c. applying a lacquer over the sheet surface;
d. embossing the product;
e. re-moisturising the underside of the product;
f. rewinding the product;
g. allowing a dwell time to re-stabilise the product.

12. A method as claimed in Claim 10 or Claim 11 performed on a paper making machine immediately after the drum reel operation.

## Patentansprüche

1. Papierprodukt, umfassend eine Schicht aus leicht gefärbtem Basispapier, mit einer oberen Oberfläche, bei welchem ein Teilstück der Schicht unter der oberen Oberfläche mit einer färbenden Tinte imprägniert ist, wobei die färbende Tinte in der Konzentration in einer Richtung durch die Schicht hindurch, die sich von der oberen Oberfläche weg bewegt, abnimmt, dadurch gekennzeichnet, dass die Rate der Abnahme bei der Konzentration der Tinte in einem ersten Teilstück des Papierprodukts, das näher an der oberen Oberfläche ist, größer ist, als in einem zweiten Teilstück des Papierprodukts, das von der oberen Oberfläche weiter weg ist.

2. Papierprodukt nach Anspruch 1, wobei die Konzentration der imprägnierten Tinte in einer ersten im wesentlichen linearen Rate durch das genannte erste Teilstück des Papierprodukts hindurch, das näher an der oberen Oberfläche des Produkts ist, und in einer zweiten und geringeren, im wesentlichen linearen Rate durch das genannte zweite Teilstück des Papierprodukts hindurch, das von der oberen Oberfläche weiter weg ist, abnimmt.

3. Papierprodukt nach Anspruch 1 oder 2, aus Zellulosefasern, synthetischen Fasern oder gemischten Fasern hergestellt.

4. Papierprodukt nach einem der vorhergehenden Ansprüche, bei dem sich die färbende Tinte im wesentlichen quer über den gesamten Oberflächenbereich des Papierprodukts erstreckt.

5. Papierprodukt nach einem der vorhergehenden Ansprüche, fähig oder geeignet, so gefaltet zu werden, dass ein Falz in dem Produkt gebildet wird, derart, dass die resultierende Beschädigung der äußersten Fasern nach der oberen Oberfläche hin nicht zuläßt, dass sich ungefärbte Fasern zeigen.

6. Papierprodukt nach einem der vorhergehenden Ansprüche, bei dem die leicht gefärbte Papierbasis Tinte aufweist.

7. Papierprodukt nach einem der vorhergehenden Ansprüche, mit mehr als einer Papierschicht, wobei die färbende Tinte nur in der oberen Schicht vorhanden ist.

8. Papierprodukt nach einem der vorhergehenden Ansprüche, bei dem die färbende Tinte ausgewählt ist, eine oder mehrere der folgenden Charakteristiken aufzuweisen:
a) hoher Widerstand gegenüber trockenem und feuchtem Abreiben;
b) hoher Widerstand gegenüber Farbänderung unter Druck und Temperatur;
c) Flexibilität des Tintenfilms beim Prägen und Einhängen, um das Reißen der Tintenschicht zu verhindern;
d) gute Folienstempelungs-, Blinddruck- und Siebdruck-Eigenschaften;
e) gute Lichtechtheit (d. h. Widerstand gegenüber Verblassen, zum Beispiel 3 Min. auf der Blue Wool Scale);
f) kein Abschmieren auf die Unterseite;
g) kein Abschmieren auf die Design-Walzen oder Matrizen-Walzen;
h) gute Papierdurchdringungs-Charakteristiken.

9. Papierprodukt nach einem der vorhergehenden Ansprüche, bei dem die färbende Tinte bis auf eine Tiefe von mindestens 30 Mikron unter die obere Oberfläche des Papierprodukts eindringt.

10. Verfahren zum Herstellen eines Papierprodukts, folgende Schritte einschließend:
a) Bedrucken einer Blattoberfläche des Papierprodukts mit Tinte;
b) Eindringenlassen der Tinte in ein Teilstück des Papierprodukts unter der Blattoberfläche sowie
c) erneutes Bedrucken des Blatts mit Tinte, so dass die Rate der Abnahme bei der Konzentration der Tinte in einem ersten Teilstück des Papierprodukts, das näher an der oberen Oberfläche ist, größer ist als in einem zweiten Teilstück des Papierprodukts, das von der oberen Oberfläche weiter weg ist.

11. Verfahren nach Anspruch 10, ferner einen, oder mehrere, der folgenden Schritte einschließend:
a) Abwickeln des Papierprodukts;
b) Trocknen der Tinte zwischen den zwei Druckaufbringungen;
c) Aufbringen eines Lacks über die Blattoberfläche;
d) Prägen des Produkts;
e) erneutes Befeuchten der Unterseite des Produkts;
f) erneutes Wickeln des Produkts;
g) Zulassen einer Verweilzeit zum Restabilisieren des Produkts.

12. Verfahren nach Anspruch 10 oder 11, auf einer Papierherstellungsmaschine, unmittelbar nach dem Trommel-Haspel-Vorgang, durchgeführt.

## Revendications

1. Produit de papier comprenant une couche de papier de base légèrement colorée, ayant une surface supérieure dans laquelle une portion de la couche en dessous de la surface supérieure est imprégnée d'une encre de coloration, dans lequel la concentration de l'encre de coloration diminue dans une direction traversant la couche en s'écartant de la surface supérieure, caractérisé en ce que le taux de diminution de la concentration de l'encre est plus important dans une première portion du produit de papier la plus procne de la surface supérieure que dans une deuxième portion du produit de papier plus éloignée de la surface supérieure.

2. Produit de papier selon la revendication 1, dans lequel la concentration d'encre imprégnée diminue à un premier taux substantiellement linéaire à travers ladite première portion du produit de papier la plus proche de la surface supérieure du produit, et à un deuxième taux inférieur substantiellement linéaire à travers ladite deuxième portion du produit de papier plus éloignée de la surface supérieure.

3. Produit de papier selon la revendication 1 ou la revendication 2, fabriqué à partir de fibres cellulosiques, synthétiques ou mixtes.

4. Produit de papier selon l'une quelconque des revendications précédentes, dans lequel l'encre de coloration s'étend substantiellement en travers de toute la superficie du produit de papier.

5. Produit de papier selon l'une quelconque des revendications précédentes, capable de, ou prévu pour, être plié de manière à former un pli dans le produit de telle sorte que l'endommagement résultant des fibres les plus externes vers la surface supérieure ne permette pas de distinguer des fibres non colorées.

6. Produit de papier selon l'une quelconque des revendications précédentes, dans lequel la base de papier légèrement colorée est teinte.

7. Produit de papier selon l'une quelconque des revendications précédentes, ayant plus d'une couche de papier et dans lequel l'encre de coloration est présente uniquement dans la couche supérieure.

8. Produit de papier selon l'une quelconque des revendications précédentes, dans lequel l'encre de coloration est sélectionnée de manière à avoir une ou plusieurs des caractéristiques suivantes :
a. haute résistance au frottement à sec et humide;
b. haute résistance au changement de teinte sous l'effet de la pression et de la température;
c. flexibilité du film d'encre pour le gaufrage et l'emboîtement de manière à éviter la craquelure de la couche d'encre ;
d. bonnes propriétés de gravure de la feuille, d'empreinte à chaud et de sérigraphie;
e. bonne résistance à la lumière (c'est-à-dire résistance à la décoloration, par exemple 3 min sur l'échelle Blue Wool);
f. pas de maculage sur la face inférieure;
g. pas de maculage sur les rouleaux d'ébauche ou les rouleaux de matrice;
h. bonnes caractéristiques de pénétration du papier.

9. Produit de papier selon l'une quelconque des revendications précédentes, dans lequel l'encre de coloration pénètre jusqu'à une profondeur d'au moins 30 microns sous la surface supérieure du produit de papier.

10. Procédé de production d'un produit de papier comportant les étapes consistant à :
a) imprimer avec de l'encre une surface de feuille du produit de papier;
b) laisser l'encre passer dans une portion du produit de papier en dessous de la surface de la feuille; et
c) réimprimer la feuille avec de l'encre, de sorte que le taux de diminution de la concentration de l'encre soit plus important dans une première portion du produit de papier la plus proche de la surface supérieure que dans une deuxième portion du produit de papier plus éloignée de la surface supérieure.

11. Procédé selon la revendication 10, comportant également une ou plusieurs des étapes suivantes:
a. dérouler le produit de papier;
b. sécher l'encre entre les deux applications d'impression;
c. appliquer un laquage par-dessus la surface de la feuille;
d. graver le produit;
e. réhumidifier la face inférieure du produit;
f. réenrouler le produit;
g. laisser attendre pendant un temps de séjour pour restabiliser le produit.

12. Procédé selon la revendication 10 ou la revendication 11, effectué sur une machine à papier immédiatement après l'opération de l'enrouleuse à tambour.
